

# United States Patent Office

2,960,401

Patented Nov. 15, 1960

1

2,960,401

## PRECIPITATION-HARDENABLE, ALUMINUM-CONTAINING IRON BASE ALLOY

William J. Buehler, Hyattsville, and Charles G. Dalrymple, Rockville, Md., assignors to the United States of America as represented by the Secretary of the Navy

No Drawing. Filed Dec. 30, 1958, Ser. No. 783,998

6 Claims. (Cl. 75—124)

(Granted under Title 35, U.S. Code (1952), sec. 266)

The invention described herein may be manufactured and used by or for the Government of the United States of America for governmental purposes without the payment of any royalties thereon or therefor.

This invention relates to low aluminum content iron base alloys. More specifically the invention relates to low aluminum content iron base alloys containing no alloying metals in short supply but having superior strength combined with oxidation and corrosion resistance at elevated temperatures as well as acceptable static and dynamic mechanical properties at room temperature and to the process for producing these alloys.

The high temperature strength and oxidation resistance of the iron base alloys containing from 14 to 16% by weight of aluminum with 3 to 4% by weight of molybdenum have been known for some time. These alloys are, however, too brittle to permit satisfactory working at room temperatures. Iron base alloys containing 8 to 12% by weight of aluminum are sufficiently ductile to permit such working but lack good oxidation resistance and strength at elevated temperatures.

The value of the aluminum addition to the iron base to prevent oxidation at elevated temperatures has been long recognized. The addition of the aluminum, however, promotes grain growth which interferes with working at room temperatures. Carbon present is believed to segregate at the grain boundaries upon cooling forming brittle carbides surrounding the iron-aluminum grains. These carbides cause brittleness and failures due to the rapid deterioration of the carbides. Increasing the aluminum content of the alloy merely decreases the ductility by aggravating the brittleness and large grain structure. The manufacture of carbon free iron-aluminum alloys in present industrial furnaces is practically impossible. U.S. Patent No. 2,172,023 to J. D. Gat and U.S. Patent No. 2,726,952 to E. R. Morgan suggest the addition of a small proportion of a metal such as titanium, molybdenum, tantalum, columbium and the like to combine with the carbon present to form uniformly distributed fine carbides of low solubility. In this manner the carbides are distributed about the mass to form nuclei of crystallization and are removed from the iron-aluminum grain boundaries. In preparing these alloys the various metals are ordinarily melted, thoroughly commingled under conditions protecting them from excessive oxidation and, cast in the desired form. Alloys prepared in this manner have, however, been found to lack satisfactory strength and hardness at elevated temperatures.

In accordance with the present invention the disadvantages of the prior art are overcome and there is produced an iron-aluminum alloy which is sufficiently ductile to permit working at room temperatures and yet is capable of maintaining increased hardness and strength at elevated temperatures. This is accomplished by subjecting a specific iron base low aluminum content alloy containing a ternary metal to specific precipitation hardening treatments.

It is therefore an object of the present invention to

2

provide an aluminum-iron alloy containing no strategic metals in short supply which has superior strength and oxidation and corrosion resistance at elevated temperatures as well as sufficient ductility and other mechanical properties to permit working at room temperatures.

Another object is to provide a process for preparing an iron base aluminum alloy having sufficient ductility and other mechanical properties to permit the alloy to be worked at room temperatures but capable of being treated to give high strength and hardness at elevated temperatures.

A further object is to provide a process for preparing a low aluminum content iron base alloy capable of superior strength and oxidation and corrosion resistance at elevated temperatures.

Other objects and the attendant advantages of the invention will become apparent to those skilled in the art as the invention is disclosed in the following detailed description.

The above objects are accomplished in accordance with the present invention by utilizing an iron-aluminum alloy system containing from about 8% to about 12% by weight of aluminum and adding to this alloy system from about 1% to about 3.5% of a third metallic element which promotes a precipitation hardening reaction. This ternary alloy system is subjected first to a "solution treatment" to produce an alloy of suitable ductility for working at room temperature. The alloy system is then subjected to an "aging treatment" to produce an alloy having the desired strength and oxidation and corrosion resistance at elevated temperatures.

The iron base alloy systems containing from about 8 to about 12% aluminum by weight have been found satisfactory in producing the alloy of the invention, this range providing suitable room temperature ductility and good oxidation resistance at elevated temperatures. However, the iron base alloy systems found to have the most desirable characteristics are those containing about 8% by weight of aluminum.

The ternary metallic element which has been found to promote the significant precipitation hardening of the invention was titanium. From about 1% to about 3.5% of titanium must be present in the alloy system. Titanium percentages below about 1% produce too small a change in hardness and are ineffective in causing the required precipitation to occur. Titanium percentages in excess of about 3.5 percent make the alloys brittle and render them useless as a structural material.

Carbon added to the alloy combinations was found useful in producing a refined grain size but contributes little to the precipitation hardening mechanism.

Metals other than titanium also do not contribute substantially to this precipitation hardening mechanism.

The alloys of the invention may be melted by any suitable melting technique such as by electric arc or induction methods. An atmosphere of hydrogen or helium may be used in the melting chamber to prevent excessive oxidation. Air atmosphere melting may be employed providing an inert gas blanket is placed over the melt or a suitable slag cover is placed on the molten alloy.

In accordance with the process of the invention the alloy is subjected to "solution treatment" by heating to a temperature between about 900° to about 1000° C. This temperature range is critical since temperatures above 1000° C. weaken the material by causing excessive grain growth. Temperatures below 900° C. are too low to place the alloy in the single phase solution range required for precipitation hardening. The material must be held at this temperature until a single phase solution is achieved. The time the alloy must be held at this temperature varies greatly with the thickness and mass

of the material being heated and must be determined empirically. For an 0.1" thick specimen an optimum time for "solution treatment" of the alloy of the invention has been found to be about one hour or less.

After the alloy has been held at the required temperature for a sufficient period to make it a single phase solution, the alloy is quenched or cooled rapidly to room temperature. In this condition the alloys are softest and most easily formed and machined.

After forming as desired the alloy is subjected to a second heat treatment or "aging treatment." The purpose of this aging treatment is to promote the precipitation from the solid solution. The aging temperature is closely interrelated with the alloy system in question. Too high an aging temperature will promote what is called "overaging." This means that the particles precipitating from the solution grow too large and are ineffective in producing increased hardness. For the alloy of this invention the critical temperature range has been found to be between about 500° C. to about 600° C. depending upon the particular proportions of the alloy.

As with the "solution treatment" the minimum time required for "aging" the alloy depends upon the section thickness and the mass of the material being heated and therefore must be determined empirically. It is important, however, that the heating time be sufficient to insure that the entire mass is heated to a temperature within the required temperature range to produce optimum strength alloys. The constituent precipitating from the solid solution should form its own normal atomic lattice arrangement different from that of the matrix. It should form fine discrete particles that remain coherent and cause a mutual distortion of the matrix lattice near the particles. This matrix distortion is the basis for the hardening process. It has been found, however, that the alloys prepared in accordance with the process of this invention do not "overage" upon heating to 600° for prolonged periods i.e. they do not lose their increased hardness even when subjected to 600° C. for long periods.

The following table lists various alloy systems according to the invention which were given the "solution" and "aging" treatments described above. The times given were optimum for the 0.1" thick specimens tested.

ability to maintain their increased hardness for prolonged periods of time at temperatures up to 600° C. Or, stated in another way, they do not "overage" upon heating to 600° C. (1112° F.). Even when heated to 600° C. for over 100 hours the improved strength properties attained through the precipitation hardening process of the invention remained.

The higher titanium alloys i.e. those having from about 2.5 to about 3.5% by weight of titanium, also show improved strengths at temperatures up to about 800° C.

Typical room temperature tensile properties of an alloy prepared in accordance with the invention are disclosed in the following table to indicate the effects of the hardening steps of the process of the invention.

Table II

| Alloy Composition              | Heat Treatment                                        | Hardness RC | Percent Elongation <sup>1</sup> | Tensile Strength <sup>2</sup> |
|--------------------------------|-------------------------------------------------------|-------------|---------------------------------|-------------------------------|
| 1.6% Ti, 8% Al,<br>0.1% C, Fe. | As Rolled.....                                        | 16          | 7                               | 97,140                        |
| 1.6% Ti, 8% Al,<br>0.1% C, Fe. | 1,000° C., ½ hr.<br>water quench,                     | 10          | 15                              | 82,285                        |
| 1.6% Ti, 8% Al,<br>0.1% C, Fe. | 1,600° C., ½ hr.<br>water quench,<br>500° C., 1 hour. | 29          | 2                               | 111,420                       |

<sup>1</sup> Based on a gauge length of two inches.

<sup>2</sup> Pounds per square inch.

From Table II it may be seen that the alloy in the "as rolled" condition possessed intermediate strength and elongation (ductility). For minimum strength and maximum elongation the "solution treated" condition (1000° C., ½ hr., water quench) is best. This leaves the alloy in a state of maximum ductility for subsequent room temperature forming operation. Then to promote maximum strength "aging" is performed. With the "aging treatment" the elongation value drops to 2%.

From the foregoing it may be seen that there has been disclosed a low aluminum content iron base alloy system which is sufficiently ductile to permit working at room temperatures and which when properly treated is capable

Table I

| Melt No. | Aluminum=8%,<br>Iron=Remainder |           | Solution Heat Treatment |                |                       |                             | Aging Heat Treatment              |                  |                                        |
|----------|--------------------------------|-----------|-------------------------|----------------|-----------------------|-----------------------------|-----------------------------------|------------------|----------------------------------------|
|          | Percent Ti                     | Percent C | Temp.,<br>°C.           | Time,<br>hours | Quench<br>Medium      | Hardness,<br>R <sub>e</sub> | Optimum<br>Aging<br>Temp.,<br>°C. | Time,<br>minutes | Max.<br>Hardness,<br>(R <sub>e</sub> ) |
| 1.....   | 0.5                            | .....     | 900                     | 1              | Room Temp.,<br>Water. | 5.5                         | 500                               | 10               | 5.5                                    |
| 2.....   | 1.0                            | .....     | 900                     | 1              | do.....               | 7                           | 600                               | 10               | 25.5                                   |
| 3.....   | 1.5                            | .....     | 900                     | 1              | do.....               | 9                           | 600                               | 10               | 35                                     |
| 4.....   | 2.0                            | .....     | 900                     | 1              | do.....               | 9                           | 550                               | 10               | 37                                     |
| 5.....   | 2.5                            | .....     | 900                     | 1              | do.....               | 20                          | 600                               | 10               | 43                                     |
| 6.....   | 3.0                            | .....     | 900                     | 1              | do.....               | 18                          | 600                               | 10               | 47                                     |
| 7.....   | 3.5                            | .....     | 900                     | 1              | do.....               | 15                          | 600                               | 20               | 46                                     |
| 8.....   | 0.8                            | 0.05      | 900                     | 1              | do.....               | 3                           | 500                               | 10               | 9                                      |
| 9.....   | 1.3                            | 0.05      | 900                     | 1              | do.....               | 5.5                         | 500                               | 10               | 17                                     |
| 10.....  | 1.8                            | 0.05      | 900                     | 1              | do.....               | 7.5                         | 500                               | 10               | 30.5                                   |
| 11.....  | 2.3                            | 0.05      | 900                     | 1              | do.....               | 10                          | 570                               | 10               | 35                                     |
| 12.....  | 2.8                            | 0.05      | 900                     | 1              | do.....               | 15                          | 600                               | 10               | 38.5                                   |
| 13.....  | 3.3                            | 0.05      | 900                     | 1              | do.....               | 18.5                        | 600                               | 10               | 42                                     |
| 14.....  | 1.1                            | 0.1       | 900                     | 1              | do.....               | 3                           | 500                               | 10               | 9                                      |
| 15.....  | 1.6                            | 0.1       | 900                     | 1              | do.....               | 10                          | 530                               | 10               | 29                                     |
| 16.....  | 2.1                            | 0.1       | 900                     | 1              | do.....               | 11                          | 550                               | 10               | 31                                     |
| 17.....  | 2.6                            | 0.1       | 900                     | 1              | do.....               | 15                          | 600                               | 10               | 37                                     |
| 18.....  | 3.1                            | 0.1       | 900                     | 1              | do.....               | 18.5                        | 600                               | 10               | 42                                     |
| 19.....  | 8.6                            | 0.1       | 900                     | 1              | do.....               | 19                          | 600                               | 10               | 45                                     |

From the foregoing it may be seen that iron base alloys containing about 8% by weight of aluminum and which contain as a ternary addition element from about 1% to about 3.5% by weight of titanium have been found to be capable of precipitation hardening when subjected to heat treatments in accordance with the process of the invention as disclosed above. These treated alloys have the

ability to maintain their increased hardness for prolonged periods of time at temperatures up to 600° C. There has also been disclosed a process for producing the alloy described.

Within the scope of the appended claims it is understood that the invention may be practised otherwise than as specifically disclosed.

What is claimed as new and desired to be secured by Letters Patent of the United States is:

1. A structural material which is sufficiently ductile to permit working at room temperatures and capable upon further heat treatment of high strength and oxidation resistance at elevated temperatures consisting essentially of a mixture of from about 8% to about 12% by weight of aluminum, from about 1% to about 3.5% by weight of titanium and the remainder iron, said mixture being a supersaturated solid solution and being further characterized by a Rockwell hardness of about 7 to about 20, and a tensile strength of about 80,000 pounds per square inch.

2. A structural precipitation hardened material capable of high strength and oxidation resistance at elevated temperatures consisting essentially of a mixture of from about 8% to about 12% by weight of aluminum, from about 1% to about 3.5% by weight of titanium and the remainder iron, said mixture being characterized by a Rockwell hardness of about 25 to about 47, and a tensile strength of about 110,000 pounds per square inch.

3. The method of producing a low aluminum content iron base alloy material having sufficient ductility to permit working at room temperatures and capable upon further heat treatment of high strength and oxidation resistance at elevated temperatures by heating a mixture consisting essentially of from about 8% to about 12% by weight of aluminum, from about 1% to about 3.5% by weight of titanium and the remainder iron to a temperature between about 900° C. and 1000° C. until said mixture becomes a single phase solution and subsequently rapidly cooling said solution to produce a supersaturated solid solution.

4. The method of producing a low aluminum content

iron base alloy material having high strength and oxidation resistance at elevated temperatures by heating a mixture consisting essentially of from about 8% to about 12% by weight of aluminum, from about 1% to about 3.5% by weight of titanium and the remainder iron to a temperature between about 900° C. and 1000° C. until said mixture becomes a single phase solution, rapidly cooling said solution to produce a supersaturated solid solution and subsequently heating said solid solution to a temperature between about 500° C. and 600° C. to cause aging.

5. A precipitation-hardened article made of an alloy consisting essentially of about 8-12% aluminum by weight, about 1-3.5% titanium by weight, and the remainder iron.

6. A solution-treated article made of an alloy consisting essentially of about 8-12% aluminum by weight, about 1-3.5% titanium by weight, and the remainder iron, said article being characterized by sufficient ductility to permit working at room temperatures and further characterized by high strength and oxidation resistance at high temperatures.

References Cited in the file of this patent

UNITED STATES PATENTS

|           |                |               |
|-----------|----------------|---------------|
| 2,172,023 | Gat            | Sept. 5, 1939 |
| 2,726,952 | Morgan et al.  | Dec. 13, 1955 |
| 2,768,915 | Nachman et al. | Oct. 30, 1956 |
| 2,859,143 | Nachman et al. | Nov. 4, 1958  |

OTHER REFERENCES

Comstock: Titanium in Iron and Steel, 1955, pages 231-234, published by John Wiley and Sons, Inc., New York, N.Y.